

## UNITED STATES PATENT OFFICE

2,238,738

COMPOSITION FOR COATING METAL BEING  
FORMED

Harold R. Hurd, Independence, Mo.

No Drawing. Application July 24, 1939,  
Serial No. 286,155

5 Claims. (Cl. 252—18)

This invention relates to a new composition of matter for coating metals being formed and particularly to that type of a preparation which serves to facilitate rapid and accurate forming of the metals.

In the various methods of changing the forms of metal, such as wire drawing, stamping, die casting, etc., it has been the general practice to use some lubricant to lessen the friction between the metal being formed and the tools or dies by which the forming is being accomplished. The most common lubricant now being used for the cold drawing of metals, consists of a composition of tallow and talc, while in the hot drawing, graphite is generally used.

The present invention contemplates the production of a new preparation that will materially lessen the power usually required to perform the metal forming operation; will permit of a material increase in production; and will cause the metal product to have a much smoother finish than is obtainable by the use of the now known lubricants.

The ingredients entering into this preparation include a vegetable soap, ferrous oxide and lime water.

The vegetable soap may include soaps containing various kinds of vegetable oils, such as olive oil, cottonseed oil, peanut oil, corn oil, etc., however, the soap well suited for the present composition contains considerable cottonseed oil treated with any suitable caustic alkali. The ferrous oxide (FeO) is the standard commercial product.

The lime water is a saturated solution of calcium hydroxide with water.

Various preparations for different uses may be had by intermixing the ingredients in the following proportions, by weight: 28 to 78 parts of a vegetable soap; 2 to 4 parts of ferrous oxide; and 20 to 70 parts of lime water.

For use in drawing the heavier steel wire, the following proportions, by weight of the ingredients, has been found very satisfactory: 78 parts of vegetable soap; 2 parts of ferrous oxide; and 20 parts of lime water.

A composition for drawing the finer steel wires, the following proportions of the ingredients has been used with very satisfactory results: 56 parts of vegetable soap; 4 parts of ferrous oxide; and 40 parts of lime water.

For drilling and cutting operations in steel, the following composition has been found best suited: 28 parts of vegetable soap; 2 parts ferrous oxide; and 70 parts lime water.

Many other variations of the composition with range of proportions above recited, might be made to meet the various needs encountered in forming iron products by extruding die casting, die forming, or cutting.

The composition is applied to the metal parts, to be formed, to coat the same, so that for example, when the wire is being drawn, the wire is lubricated with the composition whereby the friction between the wire and drawing die is greatly reduced and thereby, the speed of operation can be increased. By the reduction of friction, due to better lubrication, it is evident that the life of the die is greatly increased.

10 When using this composition for drawing wire, the finished wire has a highly polished finish not obtainable when using the standard lubricants; furthermore, there is a durable coating formed on the wire which serves to prevent the oxidation of the steel.

15 After many tests, it is very evident that this composition so coats the wire being formed that the die surfaces also receive a smooth coating, thus insuring the passing of the wire through the die with a lubricating coat therebetween, which prevents to a large degree, the undesirable heating of the die and the wire.

20 It is apparent that by the use of this new composition of matter, the operation necessary in forming iron products may be facilitated and the product will be materially improved.

25 Having thus described the invention, what is claimed as new and desired to be secured by Letters Patent is:

30 1. A composition of matter for coating metals being formed, resulting from intermixing the following ingredients in the following proportions, by weight, namely: 28 to 78 parts of a vegetable soap; 2 to 4 parts of ferrous oxide; and 20 to 70 parts of lime water.

35 2. A composition of matter for coating metals being formed, resulting from intermixing the following ingredients in the following proportions, by weight, namely: 78 parts of a vegetable soap; 2 parts of ferrous oxide; and 20 parts of lime water.

40 3. A composition of matter for coating metals being formed, resulting from intermixing the following ingredients in the following proportions, by weight, namely: 56 parts of a vegetable soap; 4 parts of ferrous oxide; and 40 parts of lime water.

45 4. A composition of matter for coating metals being formed, resulting from intermixing the following ingredients in the following proportions, by weight, namely: 28 parts of a vegetable soap; 2 parts of ferrous oxide; and 70 parts of lime water.

50 5. A composition for coating material which is to be submitted to a drawing operation in the manufacture of wire, comprising a dispersion of lime and ferrous oxide in water stabilized by means of a vegetable oil soap.